

Sept. 1, 1936.

W. BOWKER ET AL

2,052,602

CELLULOSE ACETATE MATERIAL FOR PLAYING CARDS, ETC

Filed May 18, 1934



INVENTORS  
BJORN ANDERSEN AND  
WILLIAM BOWKER

BY  
MELVIN A. LEVINE  
ATTORNEY

## UNITED STATES PATENT OFFICE

2,052,602

CELLULOSE ACETATE MATERIAL FOR  
PLAYING CARDS, ETC.William Bowker, Newark, and Bjorn Andersen,  
Maplewood, N. J., assignors to Celluloid Corporation,  
a corporation of New Jersey

Application May 18, 1934, Serial No. 726,238

5 Claims. (Cl. 18—57)

This invention relates to card material such as playing cards and the like and to the method of manufacturing the same, wherein the base or body of the playing card contains cellulose acetate or other organic derivative of cellulose.

An object of the invention is the economic and expeditious production of card materials such as playing cards, having a base containing cellulose acetate, which are opaque, springy or full of life and are of low specific gravity. Other objects of the invention will appear from the following detailed drawing and specification.

Playing cards made from cellulosic plastics have been known for many years but they never attained commercial success because they were too heavy, that is, they had a too high specific gravity when made sufficiently opaque. Card material made according to this invention, however, is at least as opaque and light as the ordinary type of filled paper cards and has the further advantage of having more life or "snap", a property much desired by card players. Further, the cards formed according to this invention do not, upon use, wear down or peel to exhibit a fabric material that is soft and absorbent of liquids, etc. The cards may be washed without hazard of destroying their opacity or snap.

Playing cards made according to the method of this invention are opaque and of relatively low specific gravity, have low shrinkage characteristics, lie flat without curling and have a snappy resilient feel to the touch. A further advantage is that the material is comparatively free from tendency to generate or retain static electricity which is characteristic of the usual cellulosic materials or paper and linen materials. Being free from the property of maintaining a static electric charge, the cards do not cause lint and dirt particles to adhere to themselves.

Heretofore, it has been impossible to make an entirely satisfactory cellulose acetate sheet material for use in playing cards. The cards have either been too heavy, too translucent or have exhibited a strong tendency to shrink and warp and have also lacked that resiliency or snap which is such a pleasing factor to the card player. We have overcome these difficulties and have produced a card which appears to be satisfactory in every respect.

According to our invention, we produce a satisfactory cellulose derivative playing card material, which has sufficient opacity and sufficiently low specific gravity so as to have a feel to the hand more like the playing card made from a paper or cloth base, and at the same time has sufficient

stiffness, resiliency and lack of brittleness to form excellent long lasting cards. Accordingly, the card material is necessarily made principally from a cellulose acetate base with or without a small addition of cellulose nitrate or pyroxylin, 5 and using as the principal pigment a very finely divided titanium dioxide combined with a plasticizer.

The cellulose acetate, preferably with an acetyl value of between 49 and 60 calculated as acetic acid, may or may not be mixed with from 5 to 15 parts of cellulose nitrate per 100 parts of cellulose acetate. It is highly desirable to incorporate this small percentage of cellulose nitrate with the cellulose acetate to obtain card material of 15 low shrinkage characteristics and at the same time obtain a material which remains perfectly flat under all atmospheric conditions. Such a small addition of cellulose nitrate, although materially enhancing the properties of the card material, influences the specific gravity of the card material with merely about .02 points raise in specific gravity, say from 1.37 to 1.39. Although we do not claim it absolutely necessary to add this small amount of cellulose nitrate to the cellulose acetate, we have found it highly desirable in spite of the slight increase in specific gravity, because of the lower shrinkage and better flatness obtained and also because it results in the cards having a snappier feel and apparently 30 more resilience to the touch.

To every 100 parts by weight of cellulose acetate and cellulose nitrate, if any cellulose nitrate be used, there may be added from 10 to 25 parts by weight of a finely divided titanium dioxide. 35 With this pigment there is obtained a maximum opacity, an excellent surface color and at the same time the low specific gravity. It is preferred to use the titanium oxide as the only pigment as other pigments used therewith are detrimental to the excellent properties of the titanium dioxide. Small amounts, as compared with the titanium dioxide, of other pigments may be used to promote in the cards properties other than opacity. To mix, for the purpose of opacity, 40 titanium oxide with other pigments like zinc oxide and zinc sulphide there is produced not only a great increase in specific gravity, but also when sufficient quantities have been employed to obtain satisfactory opacity, there is produced 45 an undesirable brittleness. To mix titanium oxide with the pigment of lower specific gravity than titanium dioxide, such as clays, aluminum silicates, etc., is also detrimental for when satisfactory opacity is obtained with such mixtures a 50 55

brittle material will result. The quantity of titanium dioxide used will depend upon the opacity desired and the thickness of the card, the greater the thickness the less pigment required.

5 To make the card material, the cellulose derivatives are placed in a kneader to which may be also added the titanium dioxide. About 100 parts, based on 100 parts of the cellulose derivative, of volatile solvents, which may consist of equal parts 10 of ethyl alcohol, acetone and ethyl acetate, in which plasticizers have been dissolved is poured over the cellulose derivatives and titanium dioxide and the mixture kneaded say from 1 to 4 hours. The gelatinized mass may then be filtered under 15 pressure to remove foreign material, after which it may be worked on malaxating rolls until the conversion of the cellulose derivative and dispersion of the pigment is completed. The material may be taken from the rolls in the form of 20 slabs which may be stacked and pressed under heat into a solid block form. Sheets of desired thickness may be cut from the block on a planer or sheeting machine which sheets are then seasoned to remove the volatile solvents. The material may then be heat treated before finishing, 25 to remove internal stresses set up in the sheet, by heating to the softening point.

As plasticizers there may be used any of the 30 high boiling solvents of low volatility as for example the aryl sulphonamids as para ethyl toloul sulphonamid, the alkyl phthalates as dimethyl phthalates, the dialkyl tartrates as dibutyl tartrate, the alkoxy esters of polybasic organic acids 35 as diethyoxy ethyl phthalate, and the polybasic organic acid esters of the mono alkyl ethers of polyhydric alcohols as diethylene glycol ethyl ether ester of phthalic acid. The plasticizers may be used either alone or in combination with others. Triphenyl phosphate may also be used 40 in quantities up to about 15 parts to 100 parts of cellulose derivative as a fire retarding agent. The quantity of plasticizers employed may vary within the limits given, depending upon the flexibility desired and the quantity of pigment incorporated. 45 The more titanium dioxide the greater the amount of plasticizer. The amount of total plasticizer employed may vary from 18 to 40 parts by weight per 100 parts of the cellulose derivative in the finished product.

50 The plasticizer should be such that it is held tenaciously by the cellulose ester so as to cause a minimum shrinkage in the finished material and which will permit a thorough elimination of the 55 volatile solvents used in the processing with a minimum loss of plasticizer. It is preferable that the volatile solvents be eliminated to the extent that the residual solvent content be less than 1% in the finished material.

60 To facilitate printing, the seasoned sheets may be given a matt or printing finish or surface by pressing under heat between surfaces having an embossing desired to be transferred to the acetate sheets and then cooling under pressure, for example, a matt finish may be imparted to the material by passing same between sand blasted steel plates, or a linen finish by placing linen cloth of the desired texture on nip rolls. In place 65 of or in addition to the mechanical finishes the 70 card may be finished by chemical means. For example, a matt finish may be produced by the de-esterification of the surface by the action of alkaline solutions. A suitable surface may be obtained by dipping the seasoned sheets in a 5% 75 caustic soda solution at room temperature for 30

minutes. For a deeper etch stronger caustic solutions and higher temperatures or longer dipping periods may be employed, as for example, 5 10% caustic soda solution at 40° C. for 10 minutes. The conditions may be varied to give any 10 desired results. The caustic treatment not only improves the printing qualities of the sheet, but also tends to improve the physical characteristics with respect to resiliency, resistance to distortion, etc. Other alkaline materials may be employed 10 such as ammonia, potassium and similar hydroxides.

The card material may be printed and embossed in any suitable manner customarily employed in the printing of cellulosic ester materials. For playing cards it is preferable to print the sheets and finish with a heat and pressure treatment to set the ink. Further to preserve the permanency of the print, the material may be coated with a thin film of transparent lacquer 20 which contains but little softening agent so that when dried it will not render a stack of cards tacky in normal use. Such lacquers may contain for example pyroxylin, cellulose acetate, benzyl cellulose or ethyl cellulose or mixtures of the 25 same combined with a small amount of a natural or synthetic resin and/or a small amount of a suitable plasticizer like alkyl phthalate, aryl phosphate, etc.

In the drawing is illustrated graphically the 30 tremendous importance the pigment and type of cellulose derivative plays in regard to specific gravity of the playing card material. As ordinate is given specific gravity and, as abscissa, parts 35 of filler. The eight curves represent different formulations as follows; the minimum amount of pigment required to impart the necessary opacity being given.

| Compound               | 1    | 2    | 3    | 4  | 5   | 6   | 7   | 8   | 40 |
|------------------------|------|------|------|----|-----|-----|-----|-----|----|
| Cellulose acetate..... |      |      |      |    |     |     |     |     |    |
| Pyroxylin.....         | 100  | 100  | 100  | 90 | 100 | 100 | 90  | 100 |    |
| Plasticizer.....       |      |      |      | 30 | 30  | 30  | 30  | 30  |    |
| Camphor.....           | 27.5 | 27.5 | 27.5 |    |     |     |     |     | 45 |
| Titanium dioxide.....  |      |      |      | 15 |     |     | 7.5 | 15  |    |
| Zinc oxide.....        | 60   | 30   |      | 60 | 60  | 30  |     |     |    |

The circles on the curves indicate the pigment concentration needed to obtain sufficient opacity 50 of the playing card material, so that the figures on the playing card cannot be read through even under adverse conditions, such as when a player observes a hand in the position between his eyes and a source of bright light. Curves 1, 2 and 3 55 represent a material made of a cellulose nitrate base 1—containing zinc oxide, 2—containing zinc oxide and titanium oxide in ratio 4:1, and 3—containing a straight titanium oxide. Although these figures illustrate the tremendous advantage 60 in selection of pigments, even the best sample has a specific gravity of 1.54 which is too high for a good playing card material.

Curves 4 to 8 inclusive illustrate cellulose acetate base material. It will be seen that titanium 65 oxide filled material is the only one producing a card having a specific gravity below 1.5 such as is desired by card players. Curves 7 and 8 represent examples of playing cards having the desired properties. It will be seen that 15 parts of titanium oxide per 100 parts of cellulose derivative is all the pigment necessary to give a satisfactory opacity and this results in a card material having a specific gravity far below 1.5.

The following examples of composition for 75

forming card material having specific gravity below 1.5 are given for the purpose of illustrating the invention and not as limitations.

## Example I

| Parts             |       |
|-------------------|-------|
| Cellulose acetate | 100   |
| Plasticizer       | 20-35 |
| Titanium dioxide  | 10-25 |

## Example II

| Parts             |       |
|-------------------|-------|
| Cellulose acetate | 95-85 |
| Cellulose nitrate | 5-15  |
| Plasticizers      | 20-35 |
| Titanium dioxide  | 10-25 |

To either of these formulae is added sufficient low boiling solvent to form the desired working consistency and the same are processed as more fully set out above.

It is, of course, understood that this improved material is not limited to playing cards, but finds wide application in all cases where a thin material of high degree of opacity and of relative non-shrinking and non-warping characteristics are desired. Such applications are in printing and lithographic work, mathematical and precision instruments and for veneering purposes, etc. Any desired color effects may be obtained by adding dyes or pigment colors to the titanium dioxide. The card material may be finished to any suitable thickness, for example, from .001 of an inch to 0.2 of an inch or greater. For playing card material, the thickness is preferably between 0.008 to 0.012 inch.

If desired, the cellulose acetate in the above formulations may be replaced in whole or in part by other organic derivative of cellulose, such as cellulose formate, cellulose propionate, cellulose butyrate or other organic esters of cellulose, or

ethyl, methyl or benzyl cellulose or other cellulose ethers.

It is to be understood that the foregoing detailed description and drawing are merely given by way of illustration and many alterations may be made therein without departing from the spirit of our invention.

Having described our invention what we desire to secure by Letters Patent is:

1. Opaque sheet material having a specific 10 gravity of less than 1.5 and containing cellulose acetate, cellulose nitrate in such proportion as to inhibit curling, plasticizers for the same, and titanium dioxide.

2. Opaque sheet material having a specific 15 gravity of less than 1.5 and containing cellulose acetate, cellulose nitrate in such proportion as to inhibit curling, plasticizers for the same and titanium dioxide in an amount equal to from 10 to 25% based on the weight of the cellulose derivatives present.

3. Opaque sheet material having a specific 25 gravity of less than 1.5 and containing 85-95 parts by weight of cellulose acetate, 5-15 parts by weight of cellulose nitrate whereby curling is inhibited, 25-35 parts by weight of plasticizers for the said cellulose derivatives and 10-25 parts by weight of titanium dioxide.

4. A playing card comprising opaque sheet material having a specific gravity of less than 1.5 30 and containing cellulose acetate, cellulose nitrate in such proportion as to inhibit curling, plasticizers for the same, and titanium dioxide.

5. A playing card comprising opaque sheet material having a specific gravity of less than 1.5 35 and containing cellulose acetate, a plasticizer therefore, and titanium dioxide, the surface only of the card being de-esterified.

WILLIAM BOWKER.

BJORN ANDERSEN.

40